



US005407625A

**United States Patent** [19]**Travelute et al.**[11] **Patent Number:** **5,407,625**[45] **Date of Patent:** **Apr. 18, 1995**[54] **METHOD OF FORMING SELF-TEXTURING FILAMENTS AND RESULTING SELF-TEXTURING FILAMENTS**[75] Inventors: **Fred L. Travelute, Charlotte, N.C.; Robert E. Hoffman, Catawba, S.C.**[73] Assignee: **Wellman, Inc., Shrewsbury, N.J.**[21] Appl. No.: **156,237**[22] Filed: **Nov. 22, 1993**[51] Int. Cl.<sup>6</sup> ..... **D01D 5/24; D02G 1/00**[52] U.S. Cl. ..... **264/168; 264/173; 264/177.14; 264/209.1; 264/209.3; 264/210.5; 264/210.8; 264/211.15; 264/211.17; 264/342 RE**[58] Field of Search ..... **264/168, 173, 177.14, 264/209.1, 209.3, 209.4, 209.5, 210.5, 210.8, 211.14, 211.15, 211.17, 342 RE**[56] **References Cited****U.S. PATENT DOCUMENTS**

- |           |         |                  |       |           |
|-----------|---------|------------------|-------|-----------|
| 3,663,683 | 5/1972  | Czernas et al.   | ..... | 264/346   |
| 4,035,879 | 7/1977  | Schippers        | ..... | 264/168 X |
| 4,082,731 | 4/1978  | Knopka           | ..... | 528/305   |
| 4,301,102 | 11/1981 | Fernstrom et al. | ..... | 264/168 X |
| 4,562,029 | 12/1985 | Black            | ..... | 264/167   |
| 4,803,036 | 2/1989  | Maruhashi et al. | ..... | 264/526   |

5,069,843 12/1991 Hansen ..... 264/103

**FOREIGN PATENT DOCUMENTS**

1583486 9/1990 U.S.S.R. ..... 264/210.5

**OTHER PUBLICATIONS**

English Translation of U.S.S.R. 1,583,486 (Published Aug. 7, 1990).

Translation of Japan 44-20,497 (Published Sep. 3, 1969).

*Primary Examiner*—Leo B. Tentoni*Attorney, Agent, or Firm*—Bell, Seltzer, Park & Gibson

[57]

**ABSTRACT**

A method is disclosed of producing self-texturing filaments that exhibit a desirable tendency to coil rather than to bend sharply or zig zag. The method comprises directing a quenching fluid at extruded hollow filaments of a liquid polymer predominantly from one side of the hollow filaments to thereby produce hollow filaments with different orientations on each side. Thereafter the temperature of the hollow filaments is raised to a temperature sufficient for the filaments to relax, but less than the temperature at which the filaments would shrink.

**25 Claims, No Drawings**

**METHOD OF FORMING SELF-TEXTURING FILAMENTS AND RESULTING SELF-TEXTURING FILAMENTS**

**FIELD OF THE INVENTION**

The present invention relates to self-texturing filaments formed from synthetic polymer materials, and in particular relates to a self-texturing filament formed from polyester that exhibits a desirable tendency to coil rather than to bend sharply.

**BACKGROUND OF THE INVENTION**

Synthetic polymers are used in many textile applications to replace natural textile materials such as wool and cotton. Synthetic polymers are also used for other textile-related applications such as insulation layers in clothing, particularly clothing for outdoor use in colder weather, and for bulking properties in pillows and other such products in which these properties are alternatively provided by natural materials such as feathers or by synthetic foam materials.

The starting product for almost all synthetic textile materials is a liquid polymer that is extruded in the form of a thin filament of the material. Such filaments have some immediate uses such as fishing line. In textile applications, however, synthetic filaments and the fibers and yarns made from them should desirably provide properties similar to those of natural fibers such as wool or cotton. In order to provide such properties, synthetic filaments must be textured before being formed into yarns and fabrics. As is well understood in the textile industry, texturing can comprise crimping, looping, or otherwise modifying continuous filaments to increase their cover, resilience, abrasion resistance, warmth, insulation properties, and moisture absorption, or to provide a somewhat different surface texture.

Typical texturing methods include false twist texturing, mechanical texturing such as edge crimping or gear crimping, air jet crimping, knit-de-knit crimping, and the stuffer box method. In quite logical fashion, the resulting characteristics of the textured filament reflects the texturing method used. Thus, textured filaments can take the form of entangled filaments, multifilament coils, monofilament coils, stuffer box crinkles, knit-de-knit crinkles, or core-bulked filaments. Each of these has its own particular properties, advantages, and disadvantages.

Among these various types of textured filaments, coils are preferred for certain applications such as cushions and insulation. Coiled filaments tend to give more volume and fewer sharp bends, "zig-zags," or "knees." Generally speaking, coiled filaments, and the yarns made from them, take on a coil or spiral configuration that is somewhat more three dimensional than other textured filaments and thus are preferred for many bulked applications, including those mentioned above.

Typical methods for coiling filaments include false twisting or edge crimping, both of which techniques are well-known to those of ordinary skill in the art, and will not be otherwise further described herein.

Both of these methods have various advantages and disadvantages in producing coiled yarns. For example, false twist coiling requires a conventional false twist winding system, while an edge crimp method requires the mechanical devices necessary to physically produce the crimp.

Alternatively, coiled filaments can be formed from bilateral fibers that coil following further processing. Traditionally, bilateral fibers are formed from two different generic fibers or variants of the same generic

- 5 fiber extruded in a side-by-side relationship. Although side-by-side or "bicomponent" spinning offers certain advantages, it also is a relatively demanding process that requires more complex spinning equipment and thus is advantageously avoided where unnecessary.
- 10 Therefore, it is an object of the present invention to provide a method of coiling filament, particularly polyester filament, to produce a coiled filament from which appropriate yarns or bulk material can be produced. Furthermore, it is an object of the invention to do so 15 without the requirement of false twisting, mechanical crimping, or bicomponent spinning.

**SUMMARY OF THE INVENTION**

The invention is a method of producing self-texturing filaments that exhibit a desirable tendency to coil rather than to bend sharply, "knee," or zig-zag. The method comprises directing a quenching fluid at extruded hollow filaments of a liquid polymer predominantly from one side of the hollow filaments to thereby produce hollow filaments with different orientations on each side. Thereafter, the temperature of the hollow filaments is raised sufficiently for the filaments to relax, but less than the temperature at which the filaments would shrink, to thereby prevent the filaments from crimping.

25 30 When these filaments are drawn and then permitted to relax, they coil favorably in a manner that would have otherwise required mechanical texturing.

In another aspect, the invention comprises a method of coiling bilateral hollow filaments in which the two component polymers are identical except for their degree of orientation. In yet another aspect, the invention comprises a coiled bilateral hollow polymeric filament in which the two component polymers are identical except for their degree of orientation.

35 40 The foregoing and other objects of the invention will be understood more clearly when taken in conjunction with the detailed description which follows.

**DETAILED DESCRIPTION**

The present invention is a method of producing self-texturing filaments that exhibit a desirable tendency to coil rather than to bend sharply, knee, or zig-zag. These shapes are hereinafter referred to as "crimps" or "crimping" as opposed to coils or coiling. The method comprises directing a quenching fluid at extruded hollow filaments of a liquid polymer predominantly from one side of the hollow filaments to thereby produce hollow filaments with different orientations on each side. Thereafter, the temperature of the hollow filaments is raised sufficiently for the filaments to relax while concurrently maintaining the filaments at a constant length to thereby prevent the filaments from shrinking and becoming brittle, both of which would inhibit drawability.

50 55 60 As used herein and in this art, orientation refers to the degree to which the chain molecules of a polymer are parallel to one another and to the longitudinal dimension of a filament. The degree of orientation can be measured using techniques well known in this art, particularly including birefringence.

In preferred embodiments, the liquid polymer comprises polyester which is extruded in the form of hollow filaments prior to the step of directing the quenching

fluid at the hollow filaments. Further to the preferred embodiments, the step of extruding the hollow filaments comprises extruding two C-shaped filament sections and directing the sections to merge shortly after they are extruded to form the hollow filament. It will be understood by those familiar with the extrusion of filaments with various cross-sections that the phrase "C-shaped" is a general way of designating two shapes which when brought together would have a hollow space in between, including shapes that would very much resemble the letter "C." It will be further understood that the invention is not limited to C-shape extruded sections or to resulting circular cross-sections, but that these shapes represent descriptive embodiments of the invention.

The preferred quenching fluid is air. In the most preferred embodiments, the air is directed at the filaments as closely as possible to the point at which the hollow filaments are extruded. When, as in preferred embodiments, the step of extruding the filaments comprises extruding the filaments from a spinneret, then the step of directing a quenching fluid comprises directing the quenching fluid at the filaments within about four inches or less of the spinneret, and most preferably within about two inches of the spinneret head.

In preferred embodiments, the step of directing the quenching flow of air comprises directing the flow of air at a rate sufficient to quench the hollow filaments, but less than a rate that would blow the filaments into contact with one another before they were quenched into solid form.

If evaluated immediately following quenching, the hollow filaments can be considered as having a "cold side" and a "hot side," the cold side being the side at which quenching was originally directed, with the hot side being the generally opposite portion of the filament. As will be well understood by those of skill in this art, the cold side will at this point be generally more oriented than the hot side. It will be further understood that the terms "cold side" and "hot side" are used for explanatory purposes and not as limitations.

As is generally the case in filament spinning, the next step is referred to as "take-up" in which the extruded quenched filaments are collected on a series of rollers for further processing or packaging. The filaments solidify under the affects of lowered temperature during the take-up step.

According to the invention, the solidified filaments are then relaxed by heating them to a temperature greater than ambient and that is sufficient for them to relax, but less than the temperature at which they would shrink. Although the inventors do not wish to be bound by any particular theory, the term "relax" as used herein refers to a process in which the density or compactness of the molecular structure increases as a result of the heating process.

Generally speaking, an appropriate temperature range for relaxing polyester filaments is between about 40°-60° C. (104°-140° F.), depending on the extent of relaxation desired, as the intensity of the treatment effect is proportional to the temperature used. The higher temperatures to be avoided are those approaching the glass transition temperature ( $T_g$ ) of polyester, approximately 68° C. (155° F.). In preferred embodiments of the invention, the relaxing step can be accomplished by heating the finishes applied to the filaments. As known to those familiar with this art, in more conventional

spinning methods, such finishes are generally added at ambient temperatures.

Following the relaxation step, the hot side of the filament has very little orientation. The cold side has some orientation, but less than it had after the stretching that occurred during the initial take-up step.

In order to produce the desired cooling, the relaxed filament is next drawn in otherwise normal fashion, and then released. The draw temperature generally approaches the glass transition temperature. The drawing step adds stress to each side of the filament with the more oriented cold side being more stressed than the less oriented hot side. In preferred embodiments using polyester, the filaments are drawn to a stress level of about 0.3 to 0.4 grams per spun denier. In this regard, one of the apparent effects of the invention is that the relaxing step decreases overall orientation, but increases relative orientation. The relaxed structure is more dense, and can crystallize faster when heated above  $T_g$  and drawn.

The drawn filaments are preferably cooled to room temperature, for example by cooling the draw rolls with circulating water. When the filament is released following drawing, both sides tend to return to their earlier condition ("recover"), but the cold side more so than the hot side, and the difference in the degree of recovery creates the desired coils. Preferably, the draw tension is released very suddenly, and as soon as possible after drawing. Similarly, because the relaxation forces are relatively moderate, interference with the filaments as they coil should preferably be avoided.

As a final step, the coiled filaments can be heat set, generally at temperatures of about 177° C. (350° F.) to produce a rigid coiled filament that is about 40% crystallized.

In another aspect, the invention comprises a method of coiling bilateral hollow filaments in which the two component polymers are identical except for their degree of orientation. As set forth in the background of the invention, bilateral filaments are usually those formed of two different polymers or two forms of a generic polymer. In the present invention, however, the two component polymers are identical and are only oriented differently as a result of the uneven quenching. The cooling method of the invention comprises raising the temperature of the hollow filaments to a temperature sufficient for the filaments to relax, but less than the temperature at which they would shrink. After a drawing step as described above, the filaments are released to coil in the absence of any control on their length.

In the preferred embodiments, the component polymers comprise polyester, specifically a single polyester, and the step of raising the temperature of the filaments sufficiently for the filaments to relax comprises raising their temperature to between about 40° C. and 60° C., depending upon the extent of relaxation desired.

Thus, in brief summary, the method steps of the invention can comprise extrusion, quenching, take-up, relaxation, drawing, release, and heat-setting.

In yet another embodiment, the invention comprises a coiled bilateral hollow polymeric filament in which the two component polymers are identical except for their degree of orientation. In preferred embodiments, the component polymers comprise polyester.

As stated earlier, the term "orientation" refers to the degree of parallelism of the chain molecules of a polymer. Although the inventors do not wish to be bound by any particular theory, the relaxation step of the pres-

ent invention appears to permit both portions of the filament, which have different orientations resulting from the uneven quenching carried out upon them, to relax by the same amount of orientation while they maintain a consistent length (because they are fused).

For example, a hollow filament or fiber according to the present invention that has one portion with an orientation number of 10 and another portion with an orientation number of 5 has a 2:1 ratio of orientations and will texture accordingly. If that filament is then relaxed by four (4) units using the method of the present invention, the resulting filament has one portion reduced in orientation from 10 to 6, and a second portion reduced from 5 to 1. The resulting relaxed filament now has an orientation ratio of 6:1 rather than 2:1 and will exhibit correspondingly different texturing properties. It will thus be easily seen that the orientation ratio between the two portions of the same filament has essentially been tripled without any mechanical activity whatsoever.

Filaments formed according to the present invention, even though self-coiling and self-texturing, can also be mechanically or otherwise textured to give additional textured properties should such be desired or necessary. The invention is thus not limited to methods in which no mechanical or other texturing steps are carried out, but instead provides a method in which such other texturing methods can be minimized or eliminated if so desired, or included if so desired.

As an additional advantage of the invention, however, the capability to produce coil without mechanical crimping permits the production of thinner-walled, hollow, coiled filaments. Specifically, because the hollow filaments will coil without mechanical crimping, their walls can be thinner than the walls required to withstand mechanical crimping. As a result, hollow filaments can be produced according to the present invention with as much as 25-35% void space (based on cross-section) compared to 15-18% void space for conventional, mechanically-crimped coiled hollow filaments. These more highly voided filaments give the same bulk properties as the less voided filaments, but at a significantly reduced weight. Stated differently, the invention provides a technique for obtaining high aspect ratio hollow filaments with lighter weight, but equivalent properties to more conventional hollow filaments.

#### EXAMPLE 1

An 80-pound sample of a spirally-coiled filament of 8 denier per filament (dpf) was produced on a 463-hole hollow pack using polyester. A quench cabinet was set to direct air at the filaments two inches below the spinneret at a 600 foot per minute peak air velocity. The takeup was set to standard conditions for 28/8 (spun denier/finished denier) hollow filament.

As part of the drawing process, a pre-bath and feed rolls were heated to 155° F. and the fiber was drawn at a 3.8 draw ratio. The fiber was allowed to relax exit the draw nip roll where the crimp formed. The crimp tow accumulated at this point, was fed to a cutter, and then collected in bags. The cut fiber was taken to a dryer and heat set at 350° F. after which a soft hand finish was applied.

#### EXAMPLE 2

A 463-hole pack was again utilized in the manner described in Example 1. Polyester was spun at 900 meters per minute and 171 pounds per hour throughput to

give 28 denier filaments. The same spacer length and quench profile as in Example 1 were again utilized.

For drawing, the pre-bath and feed rolls were heated to 155° F. and the draw ratio was set to 3.33. The water spray above the feed rolls was used at a relatively low flow rate and the draw rolls were cooled to ambient temperature with circulating water, and a draw nip roll was installed.

The drawn tow was taken through the dancer rolls and into the crimper with the pre-crimper steam chest off. The crimper flapper was up and the crimper nip roll pressure was reduced to 30 psi from 80 psi. The crimp formed exit the crimper nip and the crimped tow was guided onto the conveyer to the dryer. After passing through the dryer at 350° F., soft hand finish was applied and the fiber was cut on the production cutter.

Several hundred pounds of coiled filament were produced in accordance with Example 2. The material was evaluated by garnetting to form standard and queen size pillows. In spite of the soft hand finish, the material processed well and demonstrated excellent fill power. Queen pillows which normally require between 25 and 26 ounces of fill required only 22 ounces of the material according to the present invention to maintain the normal pillow size. Similarly, a test with standard pillows indicated that 16 ounces of the material of the present invention was adequate in a pillow that normally required 20 ounces of filler.

In the specification, typical preferred embodiments of the invention had been disclosed and, although specific terms have been employed, they have been used in the generic and descriptive sense only and not for purposes of limitation, the scope of the invention being set forth in the following claims.

That which is claimed is:

1. A method of producing self-texturing filaments that exhibit a desirable tendency to coil rather than to bend sharply or zig zag, the method comprising:  
directing a quenching fluid at extruded hollow liquid polymer filaments predominantly from one side of the liquid hollow filaments to thereby produce solidified hollow filaments with different orientations on each side;  
thereafter raising the temperature of the solidified hollow filaments to a temperature sufficient for the filaments to relax but less than the temperature at which the filaments would shrink.
2. A method according to claim 1 and further comprising the step of extruding a liquid polymer in the form of hollow filaments prior to the step of directing the quenching fluid at the hollow filaments.
3. A method according to claim 2 wherein the step of extruding the hollow filaments comprises extruding two C-shaped filament sections and directing the sections to merge shortly after they are extruded to form the hollow filament.
4. A method according to claim 1 wherein the step of directing a quenching fluid comprises directing air at the filaments.
5. A method according to claim 1 wherein the step of directing a quenching fluid comprises directing the fluid at the filaments close to the point at which the hollow filaments are extruded.
6. A method according to claim 2 wherein:  
the step of extruding the filaments comprises extruding the filaments from a spinneret; and

the step of directing a quenching fluid comprises directing the fluid at the filaments within about 4 inches or less of the spinneret.

7. A method according to claim 6 comprising directing the fluid at the filaments within about 2 inches of the spinneret.

8. A method according to claim 1 and further comprising the steps of:

drawing the relaxed hollow filaments; and  
releasing the drawn filaments to coil in the absence of  
any control of their length.

9. A method according to claim 8 and further comprising cooling the taken-up filaments to ambient temperature prior to the step of relaxing the filaments.

10. A method according to claim 1 wherein the step of raising the temperature of the hollow filaments to a temperature sufficient for the filaments to relax comprises raising the temperature to less than the glass transition temperature of the polymer.

11. A method according to claim 9 and further comprising heat setting the coiled filaments following the step of releasing the filaments.

12. A method according to claim 11 comprising heat setting the coiled filaments to approximately the maximum crystallization temperature of the polymer.

13. A method according to claim 12 comprising heat setting the filaments at about 350° F.

14. A method of producing self-texturing polyester filaments that exhibit a desirable tendency to coil rather than to bend sharply or zig zag, the method comprising:  
extruding liquid polyester from a spinneret in the form of liquid hollow filaments;  
directing a quenching fluid at the extruded liquid hollow filaments predominantly from one side of the filaments to thereby produce a solidified hollow filament with different orientations on each side;

thereafter raising the temperature of the solid hollow filaments to a temperature sufficient for the filaments to relax but less than the temperature at which the filaments would shrink;  
drawing the relaxed filaments; and thereafter  
releasing the drawn filaments to coil in the absence of any control of their length.

15. A method according to claim 14 wherein the step of extruding the hollow filaments comprises extruding two C-shaped filament sections and directing the sections to merge shortly after they are extruded to form the hollow filament.

16. A method according to claim 14 wherein the step of directing a quenching fluid comprises directing the fluid at the filaments close to the point at which the hollow filaments are extruded.

17. A method according to claim 14 wherein the step of directing a quenching fluid comprises directing the fluid at the filaments within about 4 inches or less of the spinneret.

18. A method according to claim 17 comprising directing the fluid at the filaments within about 2 inches of the spinneret.

19. A method according to claim 14 wherein the step of raising the temperature of the filaments sufficiently for the filaments to relax comprises raising their temperature to between about 40° C. and 60° C.

20. A method according to claim 14 wherein the step of directing a quenching flow of air comprises directing a quenching flow of air at a rate sufficient to quench the hollow filaments, but less than a rate that would blow the filaments into contact with one another before they were quenched into solid form.

21. A method according to claim 14 and further comprising heat setting the released coiled filaments.

22. A method according to claim 21 wherein the step of heat setting the released coiled filaments comprises heat setting the filaments at about 350° F.

23. A method according to claim 14 wherein the step of raising the temperature of the hollow filaments to a temperature sufficient for the filaments to relax comprises adding a heated liquid finish to the filaments in which the finish has been heated sufficiently to in turn raise the temperature of the hollow filaments to a temperature sufficient for the filaments to relax.

24. A method of coiling drawn bilateral hollow filaments in which the two component polymers are identical except for their degree of orientation, the method comprising:

raising the temperature of hollow bilateral filaments to a temperature sufficient for the filaments to relax but less than the temperature at which the filaments would shrink;  
drawing the relaxed filaments; and thereafter  
releasing the filaments to coil in the absence of any control on their length.

25. A method according to claim 24 wherein the component polymers comprise polyester and the step of raising the temperature of the filaments sufficiently for the filaments to relax comprises raising their temperature to about 40° C. and 60° C.

\* \* \* \* \*